

## UNITED STATES PATENT OFFICE

2,077,103

## BLEACHING PROCESS

Ehrhart Franz, Leipzig, Germany

No Drawing. Application February 9, 1934, Serial No. 710,527. In Germany December 28, 1933

## 5 Claims. (Cl. 8—2)

The present invention has for its object a process of bleaching organic materials by means of combinations delivering oxygen. As combinations delivering oxygen I particularly use for 5 the purpose of bleaching organic materials hydrogen peroxide and those combinations which are able to split up hydrogen peroxide in a watery solution, for example persulphates, percarbonates, permno-sulfuric acids, perborates and perphosphates. As is well known, organic fiber, both 10 natural and artificial, can be bleached in the bleaching-bath by means of such decolorants. Among the natural products it is particularly the animal, i. e. nitrogenous materials, and the vegetable materials, mostly free from nitrogen, that 15 can be ameliorated by means of such bleaching-baths. If the decolorants are used in a highly efficacious, i. e. active or actuated form, much oxygen is lost, because the decolorants spontaneously dissolve themselves in the bleaching-bath and deliver their oxygen not only for the 20 bleaching process. If, however, the bleaching solutions are stabilized or used in a stable form, the bleaching process, as is well known, is retarded very much and the bleaching effect is a 25 bad one.

For the present invention it is necessary that the material to be bleached is provided, at the 30 spots which are to be bleached, with combinations that are able to start and accelerate the bleaching process, either by depriving the originally stable bleaching solution of its stabilizing substance or by reacting upon the effect of its stabilizing substance. According to the present 35 invention this reaction takes place in the very proximity of the spots to be bleached. A deterioration of the bleaching solutions by soiling the perhaps lixiviated actuating substance can be avoided by using the bleaching-baths only for the impregnation of the material in question, or 40 by squirting or brushing the decolorant on the material to be bleached and finishing the bleaching process by leaving the material in a moist state, where it is suitable to work at a raised temperature. Of course it is possible to apply 45 actuating substances that do not tend to pass into the stabilized bleaching-bath. As the decolorant is worn out only at the spots that are really bleached, the decolorant is used up very 50 economically. As stabilizing substances for the bleaching-baths, respectively for the decolorants, those which are known hitherto are nearly all taken into account, especially, however, colloid substances, such as glue, colloid silicic acid, solutions of glucosides, tin-salts, organic combina- 55

tions such as mannite, phenols, particularly those inorganic or organic combinations which give the solution a low value of pH. As actuating substances we practicably use the well known metallic salts, efficacious as catalysts, or enzymes and ferments, for example extracts of yeast, as well as oxidases and peroxidases and finally those combinations which give solutions of a high value of pH. If a decolorant solution stabilized by an acid is used, it is very practicable 5 to charge the material with those substances which are able to increase the value of pH, for example with alkalies, alkalic carbonates, salts such as soda having an alkaline reaction, etc. If the latter are applied, it is possible to use the 10 actuating material during the preparatory treatment of the material to be bleached and to leave it partly in the same. Enzymes are found in most of the raw materials, so that it is possible to keep part of the enzymes or all of them in 15 the material to be bleached, by means of a suitable choice of the preparatory treatment.

The result of the aforesaid process is a very quick bleaching and therefore a considerable sparing of the material. It has proved unpracticable to apply decolorants that are stabilized by the adjustment to a low value of pH, as in the bleaching process with such means simultaneous reactions easily appear, which deteriorate the originally good bleaching, the material turning 20 yellow. Oxalic acid proved particularly practicable, because in this case the material cannot turn yellow. By means of oxalic acid even sensitive materials, such as wool, may be bleached in an absolutely satisfying way. Also in this case a 25 short treatment, lasting only a few minutes, of the material with the bath itself is sufficient; the bleaching process may then be finished by leaving the material in a moist and eventually warm state. This process proved particularly 30 suitable in the bleaching of woolen slivers. Instead of oxalic acid there may also be used phosphoric acid or boric acid with good success. Lactic acid and formic acid may also be applied. In order to spare the material it is practicable to 35 add, after the bath, other substances that spare the fibres, for example formaldehyde, glue, sugar, etc. It is especially worth remarking that the oxygen of the baths can be used up to an evanescent remainder, if very efficacious actuating substances are applied. Therefore it is possible to 40 apply baths of a very low percentage and to finish the bleaching process in stronger baths. The preparatory or final bleaching of the material can also take place according to any other 45

10

15

20

25

30

35

40

45

50

55

method. It is worth remarking, too, that the stabilized bleaching-baths may be warmer than the usual bleaching-baths applied in other cases, the result of it being a better soaking of the de-  
5 colorant.

To the extent to which this invention also touches upon an acid bleach, as well as a continuous bleaching process, attention is called to my copending applications entitled: Process for 10 bleaching, Serial No. 712,608, filed February 23, 1934, and Continuous bleaching process, Serial No. 712,609, filed February 23, 1934, respectively.

The following examples shall explain the process according to the present invention, but the 15 invention shall not be limited to these examples.

#### Example 1

Cotton is, as usual, washed in an alkaline bath 20 in the presence of 0.3 per cent. of hydrosulphite of sodium formaldehyde. After a short rinsing the material, which still reacts in alkaline fashion, is put into a bleaching-bath of 5 parts by weight of hydrogen peroxide a litre, stabilized by an addition of 0.03 per cent. of phosphoric acid. 25 It is suitable to bleach the material between 20 and 60° and to leave it in the bath for about 5 minutes. Then the material is squeezed off and kept at a temperature of 40°, until the bleaching process is finished.

Instead of phosphoric acid there may also be used sulphuric acid. In this case it is suitable to add to the bleaching-bath some sodium-sulphate (about 0.2 per cent.). Oxalic acid, too, may be 35 used as stabilizing substance, as well as isobutyl-naphthalene-sulpho-acid or boric acid. If instead of hydrogen peroxide perborate of sodium is used for the bleaching-bath, the quantity of the acid must be a little larger. The bleaching 40 process, however, lasts only inconsiderably longer.

#### Example 2

100 parts by weight of jute are preparatory 45 bleached with 800 parts by volume of bleaching solution obtained from 1 part by weight of chloride of lime by converting with soda solution (containing 0.6 part by weight of calcined soda) for 12-16 hours at the temperature of the room. Then the material is rinsed, as usual, some thio- 50 sulphate being added in the beginning, and edulcorated, if necessary, with a 5 per cent. oxalic acid solution. A distinct alkalic reaction of the material upon litmus-paper can still be observed. The bleaching process is now finished in a 55 bleaching-bath containing 0.5-1 per cent. of hydrogen peroxide, stabilized by 1 per cent. of sulphuric acid, an insignificant quantity of aluminium sulphate being added, if necessary. The material remains in the bath for about 10 minutes 60 at the temperature of the room and is then kept in a moist state for 3-4 hours at a slightly raised temperature.

Instead of sulphuric acid there can be used 65 phosphoric acid, isobutyl-naphthalene-sulpho-acid, oleyl-methyl-amino-ethane-sulpho-acid and acids of that kind or the salts thereof. Instead of aluminium salt there can be used a magnesium salt. In order to obtain a particularly clear, 70 white colour, a third bleaching-bath can be applied. For this purpose a bath of 0.1 per cent. of hyposulphite of sodium, 0.1 per cent. of calcined soda and 0.1 per cent. of oleine soap proved profitable. The bleaching process lasts about 20 75 minutes at a temperature of about 95°.

#### Example 3

Jute is freed from dust and then put, for several hours, into a bath containing 0.5 per cent. of purchasable hydrogen peroxide. The enzymes which are in the raw jute effect that the usually rather inactive decolorant solution produces a yellowish white material. Now the material is impregnated in a bath of 2-3 per cent. of hydrogen peroxide stabilized by an addition of oxalate of sodium, and kept at a normal or slightly raised temperature, until it is as white as possible. The first bath must not be stabilized, as solutions of such a low percentage are already stable. The second bath can also be stabilized by other combinations of a low value of pH or by colloids, such as silicic acid gelatine or by phenols, amines, etc. 15

#### Example 4

100 parts by weight of animal hair, for example 20 hair of the Angora-goat or sheep's wool, are, as usual, washed with soap and soda and well rinsed. The animal hair retains about 1 per cent. of soap. After having been made into sliver the material is put, for two minutes, into a bath of 0.5 per cent. of hydrogen peroxide and 0.03 per cent. of oxalic acid at a temperature of 40°, some oxalate being added if necessary. Then the material is flied or squeezed off and dried for a longer time at a lower temperature, or for a 25 shorter time at a higher temperature, for example by making the material pass over warm cylinders. It is worth remarking that the animal material is injured only quite insignificantly, and particularly that the loss of weight is quite 30 unimportant.

#### Example 5

100 parts by weight of hat stumps corroded, 40 as usual, by mercury salts, are put into 600 parts of a bleaching-bath of 3 per cent. of hydrogen peroxide and 1 per cent. of bitter salt (epsomite) and then kept in a moist state. The bleaching-bath is stabilized by 0.1-0.2 per cent. of lactic acid or phosphoric acid or by 0.1 per cent. of 45 mannite. The bleaching process lasts about 3 hours at a temperature of 40-50°, about 24 hours at the normal temperature in the room.

#### Example 6

100 parts by weight of wool in the form of a 50 cord are put, for 30 minutes at the normal temperature in the room, into 600 parts of a bath of 0.1 per cent. of permanganate of potassium very weakly acidulated by sulphuric acid or to which about 1 per cent. of bitter salt was added. Now the wool is dyed brown by hydrate of dioxide of manganese. Then the material is carefully rinsed and put into a bath containing 0.2-0.5 per cent. of hydrogen peroxide and 0.2 per cent. of sulphuric acid and 0.5-1 per cent. 55 of oxalate of sodium, for about 2 minutes at a temperature of 30-40°. Hereafter the material is put into a similar bath containing 2 per cent. of hydrogen peroxide and the corresponding quantity of stabilizing substance. After about 60 10-30 minutes the material is taken out of the bath, carefully rinsed and cleared in a bisulphite bath of about 1 per cent. of bisulphite of sodium and 0.6 per cent. of sulphuric acid. In order to obtain a white color of the utmost cleanliness 65 and durability it is practicable to apply an additional bath of hydrosulphite of sodium, containing about 0.1-0.3 per cent. of hydrosulphite of sodium. The bleaching process lasts about 70 3-6 hours at a temperature of 35-40°. Then the 75

material is carefully rinsed and freed from acid in the usual way.

A particular softness of the material is produced by an addition of protective colloids, for example a small quantity of glue or a small quantity of tanning substance given to the bleaching-bath. The damage done to the material which is to be bleached is considerably reduced by a preparatory treatment of the material with aldehydes, for example formaldehydes, acetaldehydes, chloraldehydes, etc., or by an addition of the aforesaid combinations to the bath.

The present bleaching process is not limited to the bleaching of fibrils. By means of this process there can as well be bleached other organic materials, such as horn, bone, resin, artificial resin, legumes, Indian corn, flour, etc. Of course the decolorant can also be applied by injection or in a similar fashion.

It is possible to bring the bleaching means on the material by impregnating. For this process a stabilized bleaching bath is taken; the material is impregnated by that, whereby it is useful to provide said material with compounds actuating the bleaching process. Or the material is impregnated by a bleaching bath stabilized as usual and than said material is given in a watery solution which contains a compound actuating the bleach.

In referring herein to stabilized hydrogen peroxide bleaching solutions I presume such solution to be substantially non-alkaline, i. e., that it does not give an alkaline reaction with litmus, because otherwise the solution cannot be stable.

Having thus described my invention what I claim and desire to secure by Letters Patent is:

1. The process which comprises the steps of applying to organic fiber to be bleached accelerators free of heavy metal, and of causing aqueous solutions of up to 3% hydrogen peroxide rendered stable by the addition of stabilizers free from heavy metal to act on said organic material, the accelerators locally activating the bleaching. 5

2. The process which comprises the steps of applying to organic fiber to be bleached accelerators free of heavy metal, and of causing aqueous solutions of up to 3% bleaching agents giving off hydrogen peroxide and rendered stable by the addition of stabilizers free from heavy metal to act on said fiber, the accelerators activating the bleaching solution applied to said fiber. 15

3. The process which consists in causing aqueous solutions of up to 3% hydrogen peroxide rendered stable by the addition of stabilizers free from heavy metal to act on organic fiber carrying enzymes as activators for accelerating bleaching. 20

4. In combination with a hydrogen peroxide bleaching solution for fibrous material, the separate application of a stabilizer for said solution and of an accelerator, the accelerator being applied to said material before it is bleached by the stabilized solution. 25

5. The process of claim 1, carried on first in a used and then continued in a fresh bleaching solution. 30

EHRHART FRANZ.